

# UNITED STATES PATENT OFFICE.

HANS GOLDSCHMIDT AND OTTO WEIL, OF ESSEN-ON-THE-RUHR, GERMANY, ASSIGNEES  
TO GOLDSCHMIDT THERMIT COMPANY, OF NEW YORK, N. Y., A CORPORATION OF  
NEW YORK.

## PROCESS OF PRODUCING CARBON-FREE FERROCHROMIUM.

1,136,669.

Specification of Letters Patent.

Patented Apr. 20, 1915.

No Drawing.

Application filed October 29, 1912. Serial No. 728,450.

To all whom it may concern:

Be it known that we, HANS GOLDSCHMIDT and OTTO WEIL, subjects of the King of Prussia, German Emperor, and residents of 5 Essen-on-the-Ruhr, in the Province of the Rhine, German Empire, have jointly invented certain new and useful Improvements in Processes of Producing Carbon-Free Ferrochromium, of which the following is a specification.

Carbon-free ferro-chromium cannot be manufactured in electrical furnaces, but only by means of the aluminothermic process. As the yields obtained by this process 15 are, however, comparatively unfavorable, the price of the carbon-free ferro-chromium is relatively high.

If chrome-iron ore which as is well known consists essentially of chromic oxide and ferric oxide or ferrous oxide is subjected to the aluminothermic reaction, the best result to be obtained, even when using a material of high percentage and working strictly according to the rules of the art, will give a 20 ferro-chromium with a yield of about 70 per cent. of the chromium contained in the raw material. Furthermore another disadvantage arises from the fact that it is not possible to always obtain perfectly uniform 25 results, even when using the same raw material. The reason for this peculiar fact seems to be a dissociation taking place within the aluminothermic mixture when burning.

Now it has been found that it is possible 30 to highly increase the yield of chromium from chrome-iron ore, as well as to always obtain uniform iron-chromium alloys by adding a certain percentage of oxide of chromium to the mixture of chrome-iron 35 ore and aluminum or other reducing metal, and then subjecting this mixture to the aluminothermic reaction. By this process it is possible to increase the yield of chromium from chrome-iron ore up to about 15 to 40 20 per cent and at the same time to produce ferro-chromium of a uniform composition.

The amount of the addition of chromic oxide which of course also increases the per-

centage of chromium in the alloy produced may be suitably chosen according to the percentage of chromium desired in the ferro-chromium to be produced.

In the preferred form of carrying out the invention the mixture of chrome-iron ore, chromic oxide and aluminum, (or other reducing metals) is, with a view to further increasing the yield, subjected to a pre-heating process up to temperatures near the smelting point of the reducing metal and preferably up to red heat and then to the 55 aluminothermic reaction.

What we claim is:

1. A process for increasing the yield of chromium in the aluminothermic manufacture of ferro-chromium from materials containing chromium which consists in adding to the ordinary aluminothermic mixture a certain amount of chromium oxide and subjecting this mass to the aluminothermic reaction.

2. A process for increasing the yield of chromium in the aluminothermic manufacture of ferro-chromium from chrome-iron ore which consists in adding to the ordinary aluminothermic mixture of chrome-iron ore 75 and reducing metal a certain amount of chromic oxide, preheating the mixture up to a temperature near the melting point of the reducing metal and subjecting this mass to the aluminothermic reaction.

3. A process for increasing the yield of chromium in the aluminothermic manufacture of ferro-chromium from chrome-iron ore which consists in adding to the ordinary aluminothermic mixture of chrome-iron ore 85 and reducing metal a certain amount of chromic oxide, preheating the mixture up to red heat and subjecting this mass to the aluminothermic reaction.

In witness whereof we have hereunto set 90 our hands in the presence of two witnesses.

HANS GOLDSCHMIDT. [L. S.]

OTTO WEIL. [L. S.]

In the presence of—

HELEN NUFER,  
ALBERT NUFER.